

## UNITED STATES PATENT OFFICE

2,173,457

## PRODUCTION OF LEAD CHROMATE, ETC.

Omar F. Tarr and Winslow H. Hartford, Baltimore, Md., assignors to Mutual Chemical Co. of America, New York, N. Y., a corporation of New Jersey

No Drawing. Application January 6, 1937,  
Serial No. 119,260

12 Claims. (Cl. 134—67)

This invention relates to improvements in the production of lead salts and particularly improvements in the manufacture of lead chromate, basic lead chromate and pigments containing these compounds as ingredients. The invention includes an improved method of preparing such compounds and the improved product so produced.

The process of the present invention enables colors of outstanding purity of tone, tinting strength and fastness to light to be produced. It offers a new procedure for controlling the analysis, color and physical properties of the resulting pigment. It also enables economical raw materials to be employed.

The improved process of the present invention makes use of insoluble lead compounds as the starting material, for example, the oxide, hydroxide, basic carbonate, carbonate, etc. It has heretofore been proposed to make use of such insoluble lead compounds in the manufacture of lead chromate, etc., but the present process utilizes such insoluble lead compounds to particular advantage.

The process of the present invention takes advantage of the fact that the so-called "insoluble" lead compounds of the general type of those mentioned above possess a definite solubility in water, which, although very small, nevertheless furnishes an amount of lead ion sufficient for the requirements of the process, as hereinafter described. Along with the solution of a small amount of lead there is also liberated from the "insoluble" lead compound, by the solution process, a certain amount of hydroxyl ion, which also plays an important part in the process. For instance, in the case of lead oxide, the reaction may be represented as follows:



We have found that if an insoluble lead compound of the type above mentioned is rapidly agitated in a large volume of water, and a mixture of an acid and a soluble chromate or bichromate is run in at a rate not exceeding the rate of solution of the lead compound, the lead compound is gradually and progressively converted into lead chromate-containing compounds, especially suitable for use as pigments; and that essentially all the lead compound can be so converted. By regulating the rate of addition, an alkaline condition is maintained throughout the process up to the point where all or essentially all of the initial lead compound, e. g. litharge, has

been used up to form lead chromate or lead chromate-containing compounds.

The nature of the reactions which take place appears to be illustrated, or capable of being formulated, by the following equations, based upon the use of lead oxide or litharge as the insoluble lead compound employed and the addition of admixed sodium bichromate and sulfuric acid:



While lead oxide, sodium bichromate and sulfuric acid are used in these equations for purposes of illustration, the invention is not limited to these particular compounds in actual practice.

It is apparent, from the above equations, that during the first half of the reaction, or the reaction represented by the first equation, the original basic lead compound is present in excess to control the pH of the solution in such a manner that the solution is always alkaline; and that during the second half of the reaction, or during the reaction represented by the second equation, basic lead chromate is likewise present to control the pH of the solution so that the solution is always alkaline, i. e., has a pH greater than 7.

With the gradual and progressive addition of the admixed acid and chromate or bichromate at a rate not exceeding the rate of solution of the lead compound, and in spite of the large excess of foreign anions present (sulfate anions in the above illustration), there can be no excess of hydrogen ion to redissolve the lead chromate and consequently no appreciable formation of an undesired lead salt (such as the sulfate) when the stoichiometrical quantities of reagents indicated by the equation are employed.

It is a novel and characteristic feature of the process of the invention that a pure lead chromate is prepared whenever a mixture of a bichromate and an acid is added in the stoichiometrical quantities indicated by the above equation to a slurry of finely divided lead compound of the above mentioned "insoluble" type in water, regardless of the acid employed in admixture with the bichromate added.

So also, basic lead chromates, and mixtures of basic lead chromates with normal lead chromate (known as "chrome oranges") may be readily prepared by this method by the use of a deficiency both of bichromate and of acid, e. g., by inter-

rupting the reaction described above when about 50% or more of the bichromate-acid mixture has been added.

Where lead chromate, or basic lead chromates, or mixtures of basic lead chromates with normal lead chromate, are desired, these are readily produced in a state of high purity and without admixed sulfate, even though a large excess of sulfate ions is present during the process. By keeping the reaction mixture continually alkaline during the process, the lead chromate (or basic lead chromate, etc.) is formed free from sulfate so long as the reaction is kept continually alkaline and the proper proportions of chromate and acid are added. Even when the reaction is stopped at the halfway point, or at a point where only part of the litharge has been converted to chromate, there is essentially no lead sulfate present when the proportions are correct, and when the chromate and acid are properly added to maintain an alkaline reaction.

The invention includes the further discovery that mixtures of lead chromates with other lead salts can be advantageously prepared, and in particular mixtures of lead chromate and lead sulfate of the types known as "lemon" or "primrose" yellow, but of improved properties. For the production of such composite lead pigments or products, an excess of acid over bichromate is employed to react with the lead compound, but the excess acid is so added that the reaction mixture is maintained alkaline throughout. When an excess of acid is thus added, it may be added separately, at the beginning of the reaction, and the bichromate-acid mixture then added, with gradual addition in each case and while maintaining the reaction mixture alkaline; or the bichromate-acid mixture may contain the desired excess of acid; or a combination of these two methods may be employed.

Thus, where mixtures of lead chromate and lead sulfate are to be manufactured, we have found that the percentage of lead sulfate in the finished product is substantially quantitatively equivalent to the excess of acid over bichromate employed, and that this is so even where the excess acid is some other acid than sulfuric acid, e. g., acetic acid; and that this result is obtained even though the excess acid is added at the start of the reaction and before the bichromate-acid mixture is added, as well as when the excess acid is present in the added bichromate-acid mixture, as long as sulfate ion is present in an amount at least equivalent to the desired amount of lead sulfate.

It is a characteristic and important advantage of the present process that it enables cheap and readily available starting materials to be used, for example, the cheapest lead compound, litharge; the cheapest bichromate, sodium bichromate; and the cheapest acid, sulfuric acid; and that it enables these to be completely and efficiently utilized for the production of lead chromate pigments.

The invention will be further illustrated by the following specific example for the production of a medium yellow pigment, the parts being by weight:

223 parts of litharge are agitated in 6,000 parts of water. A bichromate-acid mixture is prepared containing 49 parts of 100% sulfuric acid or its equivalent and 149 parts of sodium bichromate dihydrate or its equivalent in 500 parts of water. The litharge is advantageously in a finely divided condition to give the maximum rate of solution.

Rapid agitation is maintained while the acid-bichromate solution is added very slowly over a period of several hours, and this addition is so regulated as to maintain the reaction mixture alkaline throughout. If the bichromate-acid mixture is added too rapidly, the particles of litharge will become coated with a film of lead chromate and with consequent tendency for the reaction to be incomplete and an inferior product produced; but with regulated addition at a rate not exceeding the rate of solution of the litharge, such incomplete reaction and the production of inferior products can be readily avoided.

In the above example, a portion of the sulfuric acid used in the reaction mixture may be replaced by an equivalent quantity of another acid, such as acetic acid, which may, if desired, be added to the litharge at the start of the reaction. Where acetic acid is thus added, at the outset, and before the addition of the bichromate-acid mixture, it will react to form lead acetate which is soluble; but when the bichromate-acid mixture is added, the lead acetate is converted into sodium acetate without regeneration of acetic acid.

When it is desired to produce a mixed chromate-sulfate pigment, the excess of acid, whether sulfuric or some other acid, may be added at the outset and before the addition of the bichromate-acid mixture; or it can be added as a part of such mixture.

When sulfuric acid is added to the litharge-water suspension at the outset, it should be added gradually and while maintaining alkaline conditions throughout, so that the litharge does not become coated with the precipitated lead sulfate. By proceeding in this way, a regulated and desired amount of a lead sulfate is first produced and the chromate is then subsequently produced by the regulated addition of the bichromate-acid mixture. When the excess acid is first admixed with the bichromate and the resulting bichromate-acid mixture added, a mixed chromate-sulfate pigment is similarly prepared, the proportion of sulfate being controlled by the excess of acid present, regardless of whether the excess acid is sulfuric acid or some other acid, such as acetic acid, so long as sufficient sulfate radical is present in the chromate-acid mixture employed.

As a further example of the invention, for the preparation of a lemon yellow containing about 75% of lead chromate  $PbCrO_4$  and about 25% of lead sulfate  $PbSO_4$ , the procedure may be similar to that of the above example, with the quantity of acid and lead compound remaining unchanged, but with the bichromate used reduced to 111.8 parts by weight. With these proportions of reagents there is an excess of acid over bichromate, and insufficient chromate added for the formation of lead chromate from all of the litharge employed. In this case, as the bichromate-acid mixture is gradually and progressively added, both chromate and sulfate are formed progressively throughout the process.

The present process can be carried out at different temperatures since the relative solubility relations involved are not changed to any great extent by raising and lowering the temperature. Considerable variation in the color of the finished pigment may be obtained by variation of the temperature, the colors tending toward somewhat deeper tones as the temperature is raised. The use of hot solutions is of advantage where more rapid solution of the lead compound is desired.

In the first example given above, for the manu-

facture of a medium yellow pigment, the acid employed is sulfuric acid and the proportions of acid and bichromate are such as to give a substantially pure chromate pigment, without admixture 5 of any material amount of sulfate, even though sulfuric acid is used for admixture with the bichromate and even though sulfate radicals or anions are present throughout the process.

Instead of using sulfuric acid, as described in 10 this example, other acids can be used and the same or a similar pigment obtained.

In the example given above for the manufacture of a lemon yellow, which is a mixed chromate-sulfate pigment, the acid employed is also 15 sulfuric acid; but other acids can also be employed provided sufficient sulfate ion is present to produce the desired lead sulfate, and provided proper proportions of reagents are employed.

In the manufacture of medium yellow pigments 20 it is sometimes desirable to incorporate small quantities of lead sulfate in the pigment, and such amounts are conveniently obtained by adding the desired quantity of an acid to the batch before adding the bichromate-acid mixture, and 25 with a corresponding reduction in the amount of such mixture added. Where sulfuric acid is the acid thus added at the outset, lead sulfate will be first formed from part of the litharge, and the chromate will be subsequently formed from the 30 remainder of the litharge when the bichromate-acid mixture is subsequently added. The same or a similar result can be obtained by adding the excess acid (over that corresponding to the bichromate) to the bichromate-acid mixture, in 35 which case, as above pointed out, chromate and sulfate are both formed during the process.

The present invention is of more or less general application to the production of mixed chromate pigments containing the chromate admixed 40 with other insoluble lead salts, such as the molybdate, tungstate, etc., by the proper choice of reactants, e. g., by adding a soluble molybdate or tungstate to the bichromate-acid mixture, and with corresponding reduction in the amount of bichromate employed. Similarly mixed pigments 45 containing more than two admixed lead salts can be prepared, such as chromate, sulfate and molybdate, or chromate, molybdate and tungstate, etc. Alumina may be incorporated in the product 50 by replacing some of the acid by the desired equivalent of aluminum salt.

It is characteristic of the present process that it gives voluminous precipitates. The volume 55 of the precipitates obtained by the present process is much greater than that of those prepared by any process with which we are familiar. For example, 1 pound of the chromate pigment as precipitate may occupy as much as six gallons of space when settled from water. This material 60 is readily washed by decantation, but the extremely large volume of water required renders its separation by filtration more efficient. Despite the flocculence and voluminous nature of the pigment it is nevertheless readily filtered and washed.

The flocculence of the precipitate may be somewhat controlled by the character of the ions present in the reaction. Thus sulfates increase the flocculence while chlorides and excess bichromate decrease it. In addition, elevated temperatures 65 are also instrumental in decreasing somewhat the volume of the precipitate. By these means the physical properties and the color tone and strength of the product may be controlled while its chemical analysis may be controlled in the 70 manner described above.

In physical properties the products of the present invention are distinctly different from lead chromate-containing compounds prepared by any known method with which we are familiar. The particle size is very small, and therefore the pigments prepared by the present process possess extraordinary flocculence when dispersed in water, high tinting strength, high oil absorption, and a yellower mass tone than those prepared in the usual fashion.

We are aware that it has been proposed to prepare lead chromate pigments by causing sulfuric acid to react on litharge or similar lead compounds in the presence of a small amount of an acid or salt promoting the solution of the lead and with resulting production of a basic lead sulfate, and to cause such precipitated sulfate to react with a soluble chromate to convert the sulfate into chromate. The conversion of the sulfate into chromate, by such process, is not complete, and the product produced differs from the product produced by the present process. In the present process, where sulfuric acid is added first to the litharge, and lead sulfate produced, the sulfate is not subsequently converted into chromate, but the sulfate remains as such and the chromate is subsequently produced by further reaction upon the unreacted litharge. When the chromate together with its chemical equivalent of acid (for example sulfuric acid) is added 20 at the proper rate to the litharge suspension in water, at no time during the process is either normal or basic lead sulfate present regardless of the sulfate ion present.

It has also been proposed to prepare lead chromate pigments by the gradual addition of chromic acid to a suspension of litharge or similar lead compound in water and with the addition of a small amount of catalytic acid or salt, such as acetic acid, which is relied upon to dissolve the lead compound to form e. g. lead acetate which then reacts with the chromic acid, with regeneration of acetic acid. In the present process, even where acetic acid is used, it is not regenerated, but is converted into sodium acetate. The presence of acid in excess, even temporarily, tends to precipitate lead sulfate or lead chromate directly on the surface of the litharge particles and thus slow up or stop the reaction with resulting interference in the later stages of the process and the production of the desired pigment. In the present process, where acetic or other acid is employed, it is not employed as a catalytic acid for speeding up the solution of the litharge but is added for the purpose of controlling the amount 40 of lead sulfate in the finished product, as hereinbefore pointed out, and as illustrated by the following equation:



Any solvent action which the anion of the acid employed has on the litharge will serve to speed up the reaction, but the reaction when carried out in the presence of sulfate ions results in the production of lead sulfate which remains as such, or in the production of sulfate-chromate products as the product of the process, depending upon the proportions of soluble chromate, acid, and litharge employed.

The process of the present invention is particularly advantageous for the commercial manufacture of lead chromate and of lead chromate-containing pigments in that it enables the cheapest raw materials to be employed, namely, litharge, sodium bichromate and sulfuric acid.

The process of the present invention is also an advantageous method of making chromate-sulfate pigments and enables control of the sulfate content of the pigment to be obtained independently of the sulfate content of the solution. This control depends on the excess of acid over bichromate in the reaction mixture and is capable of giving exact control of the sulfate content.

By the present process it is also possible to 10 prepare a pure lead chromate in the presence of large quantities of ions such as sulfate, and without the formation of insoluble lead salts of such ions, such as lead sulfate, by regulation of the proportion of acid and bichromate employed. In 15 no other process with which we are familiar is a pure lead chromate obtained in the presence of sulfate.

In carrying out the process of the present invention, either for the production of a pure lead 20 chromate pigment, or for the production of a mixed chromate-sulfate pigment of accurately controlled proportions of chromate and sulfate, or for the production of other mixed chromate-containing pigments, an alkaline condition is 25 maintained throughout the process up to the point where all of the litharge or other "insoluble" basic lead compound employed has been used up to form either lead chromate alone, where that product is desired, or a mixture of lead 30 chromate and lead sulphate of regulated proportions, or the production of other desired mixed pigments. The process is controlled not only by maintaining an alkaline condition throughout, but by controlling the proportions of acid and bi- 35 chromate (or chromate) employed for reaction with the lead compound; and with gradual and regulated addition of the reagents so as to avoid an excess of acid and the precipitation of insoluble lead salts on the surfaces of the litharge 40 particles.

The improved pigments produced by the present process are definitely more voluminous than any other product with which we are familiar. The product is characterized by good light fastness and maintains its clear tone exceptionally well on dilution with inert fillers; and it has other advantageous properties, such as those hereinbefore pointed out.

We claim:

50. 1. The process of producing lead chromate pigments which comprises gradually adding, to a rapidly agitated suspension in water of a difficultly soluble basic lead compound of the group consisting of lead oxides, carbonates and hydroxides, a mixture of an acid and a compound of the class consisting of chromates and bichromates, in an amount and in proportions sufficient to convert the lead compound with substantial completeness into the desired pigment, the 55 said mixture being added at a rate not exceeding the rate of solution of the lead compound so as to maintain an alkaline reaction in the suspension throughout the process, the amount of water in said suspension being sufficient to permit substantially complete reaction of the difficultly soluble basic lead compound.

2. The process of producing a lead chromate pigment substantially free from sulfate which comprises gradually adding, to a rapidly agitated 70 suspension in water of a difficultly soluble basic lead compound of the group consisting of lead oxides, carbonates and hydroxides, a bichromate-acid mixture containing sulfate ions at a rate not exceeding the rate of solution of the lead compound so as to maintain an alkaline reaction in 75

the suspension throughout the process, the amount and proportions of said bichromate-acid mixture being sufficient to convert the lead compound with substantial completeness into the desired pigment, the amount of water in said suspension being sufficient to permit substantially complete reaction of the difficultly soluble basic lead compound.

3. The process of producing lead chromate pigments which comprises gradually adding, to a rapidly agitated suspension in water of a difficultly soluble basic lead compound of the group consisting of lead oxides, carbonates and hydroxides, a mixture of sodium bichromate and sulfuric acid in amount and in proportion sufficient to convert the lead compound with substantial completeness into the desired pigment, the said mixture being added at a rate not exceeding the rate of solution of the lead compound so as to maintain an alkaline reaction in the suspension throughout the process, the amount of water in said suspension being sufficient to permit substantially complete reaction of the difficultly soluble basic lead compound.

4. The method of producing a lead chromate pigment substantially free from sulfate which comprises gradually adding, to a rapidly agitated suspension in water of a difficultly soluble basic lead compound of the group consisting of lead oxides, carbonates and hydroxides, a mixture of sodium bichromate and sulfuric acid in stoichiometrical proportions and at a rate not exceeding the rate of solution of the lead compound so as to maintain an alkaline reaction in the suspension throughout the process, the amount of such bichromate-acid mixture being sufficient to convert the lead compound with substantial completeness into the desired lead chromate pigment, the amount of water in said suspension being sufficient to permit substantially complete reaction of the difficultly soluble basic lead compound.

5. The method of producing lead chromate pigments containing lead chromate and lead sulfate which comprises gradually adding, to a rapidly agitated suspension in water of a difficultly soluble basic lead compound of the group consisting of lead oxides, carbonates and hydroxides, a mixture of sodium bichromate and sulfuric acid containing an excess of acid over that corresponding to the bichromate, said mixture being added at a rate not exceeding the rate of solution of the lead compound so as to maintain an alkaline reaction in the suspension throughout the process, the amount of said acid-chromate mixture being sufficient to convert the lead compound with substantial completeness into the desired pigments, the amount of water in said suspension being sufficient to permit substantially complete reaction of the difficultly soluble basic lead compound.

6. In the production of lead chromate pigments by the gradual addition, to a rapidly agitated suspension in water of a difficultly soluble basic lead compound of the group consisting of lead oxides, carbonates and hydroxides, of a mixture of an acid and a compound of the class consisting of soluble chromates and bichromates, at a rate not exceeding the rate of solution of the lead compound so as to maintain an alkaline reaction in the suspension during such addition, the amount of water in said suspension being sufficient to permit substantially complete reaction of the difficultly soluble basic lead compound, the further improvement which comprises adding a limited and regulated amount of acid to the suspension before the addition of said chromate-

acid mixture, the amount of said acid-chromate mixture being sufficient to convert the lead compound with substantial completeness into the desired pigments.

5 7. In the production of lead chromate pigments containing lead sulfate by the gradual addition, to a rapidly agitated suspension in water of a difficultly soluble basic lead compound of the group consisting of lead oxides, carbonates and hydroxides, of a bichromate-acid mixture containing sulfate ions, at a rate not exceeding the rate of solution of the lead compound so as to maintain an alkaline reaction in the suspension throughout the process, the further improvement 10 which comprises gradually adding, in a similar manner, to the suspension, a limited and regulated amount of sulfuric acid, to convert part of the lead compound into a lead sulfate, before adding the bichromate-acid mixture to convert the remainder of the lead compound into pigment, the amount of water in said suspension being sufficient to permit substantially complete reaction 15 of the difficultly soluble basic lead compound.

8. The method of producing lead chromate pigment containing lead chromate and lead sulfate which comprises gradually adding to a rapidly agitated suspension in water of a difficultly soluble basic lead compound of the group consisting of lead oxides, carbonates and hydroxides, a mixture of a compound of the class consisting of chromates and bichromates and an acid, containing an excess of acid over that amount equivalent to the chromate or bichromate, and sulfate ion not less than that equivalent to the desired lead 30 sulfate, said mixture being added at a rate not

exceeding the rate of solution of the lead compound so as to maintain an alkaline condition in the suspension throughout the process and the amount of lead sulfate in the pigment being limited and regulated by the excess of acid over chromate or bichromate in the reacting mixture, the amount of said acid-chromate mixture being sufficient to convert the lead compound with substantial completeness into the desired pigments, the amount of water in said suspension being sufficient to permit substantially complete reaction 5 of the difficultly soluble basic lead compound. 10

9. Improved lead chromate pigments produced in accordance with the process of claim 1, said pigments being characterized by extraordinary 15 flocculence when dispersed in water, high tinting strength and high oil absorption.

10. Improved lead chromate pigments produced in accordance with the process of claim 2, said pigments being characterized by extraordinary 20 flocculence when dispersed in water, high tinting strength and high oil absorption.

11. Improved lead chromate pigments produced in accordance with the process of claim 3, said pigments being characterized by extraordinary 25 flocculence when dispersed in water, high tinting strength and high oil absorption.

12. Improved lead chromate pigments produced in accordance with the process of claim 4, said pigments being characterized by extraordinary 30 flocculence when dispersed in water, high tinting strength and high oil absorption.

OMAR F. TARR.  
WINSLOW H. HARTFORD. 35